

H. DE OLANETA.  
MANUFACTURE OF PRIMARY CELLS.  
APPLICATION FILED NOV. 26, 1919.

1,402,285.

Patented Jan. 3, 1922



Inventor

Harold de Olaneta,

By *Henry E. Becker*  
his Attorney.

# UNITED STATES PATENT OFFICE.

HAROLD DE OLANETA, OF NEW HAVEN, CONNECTICUT, ASSIGNOR TO WINCHESTER REPEATING ARMS COMPANY, OF NEW HAVEN, CONNECTICUT, A CORPORATION OF CONNECTICUT.

## MANUFACTURE OF PRIMARY CELLS.

1,402,285.

Specification of Letters Patent.

Patented Jan. 3, 1922.

Original application filed May 24, 1919, Serial No. 299,522. Divided and this application filed November 26, 1919. Serial No. 340,752.

To all whom it may concern:

Be it known that I, HAROLD DE OLANETA, a citizen of the United States, residing in New Haven, New Haven county, Connecticut, have invented certain new and useful Improvements in the Manufacture of Primary Cells, of which the following is a full, clear, and exact description.

This invention relates to the manufacture of primary cells. It pertains more especially to small dry cells such as those used in connection with pocket flash-lights, where manganeseiferous material is used as a depolarizing agent, and where the exciting solution, e. g., a solution of ammonium chlorid with or without zinc chlorid, is carried by or contained in a paste or gelatinous substance.

The invention is not limited, however, to this particular application.

My present invention has particular reference to the purification of the depolarizing material prior to its incorporation in the cell. The depolarizer may consist of or comprise one or more compounds of manganese generically designated as "manganese dioxid." The manganese material may be or contain among other things comminuted pyrolusite, or manganese ore, an artificial or recovered manganese dioxid produced by hydration, or a precipitate of manganese, as described in my application Serial No. 299,522, filed May 24, 1919, of which the present application is a division. In the following description I shall assume, for purposes of explanation only, that depolarization is to be effected by or in connection with a suitable manganeseiferous material having or susceptible of taking up a high content of oxygen for combination or other co-action with the hydrogen which is liberated in the cell.

The manganese dioxid commonly used in dry cells contains in many cases a number of impurities which have a deleterious action on the cell and shortens its life. I ascribe this to the fact that the impurities are acted upon by or soluble in the electrolyte, e. g., sal ammoniac solution, with the result that as soon as the ordinary cell is made, a local

action is set up which short-circuits the cell and drains the same while on the shelf. Of course, the rate of deterioration depends on the character of the impurities present. If, for example, iron is present in a substantial quantity, the cell will be drained in a very short time, because the iron is converted into an oxid of iron, which eventually finds its way to the zinc, and once in contact with the zinc a local action is set up. If, for further example, potash of any description, either free or neutralized, is present in the manganese dioxid, the sal ammoniac will dissolve the same and form a salt with the zinc or with any zinc salt present, setting up a deleterious local action. These deleterious substances in the manganese often include iron, copper and phosphorus, when manganese ore or pyrolusite is used. When artificial or hydrated manganese dioxid is employed, sulphur, oxids, nitrates, or chlorids will often be found, depending on the process of hydration. Where a precipitate of manganese is employed, lime, potash or the like will be present, depending upon the chemicals used for precipitation.

The above-enumerated impurities, and others, when chemically combined with the manganese, are insoluble in water, and when it is attempted to separate them out by the use of acids, for example, the result will either be that the manganese is dissolved, on the one hand, or, on the other hand, that insoluble compounds are created.

One of the primary objects of the present invention is to furnish an improved process for the manufacture of a relatively cheap but extremely efficient and satisfactory depolarizing material for primary cells, and more particularly small dry cells.

Another object of my invention is to provide a method of manufacturing cells wherein those impurities or substances in the depolarizer which set up local action or have other deleterious effects as a result of dissolution in or action on the electrolyte while the cell is not in use are eliminated prior to the assembly of the cell parts.

To these and other ends, the invention consists, in one aspect, in treating the materials from which the depolarizer of a primary cell are made, prior to the assembly 5 of the cell, with a solution containing one or more of the salts used in the exciting solution or paste of the battery (and preferably of approximately the same concentration), whereby all deleterious impurities soluble in 10 the exciter are removed prior to the assembly of the cell.

More specifically, my invention consists in the improvement in the manufacture of dry cells having a manganiferous depolarizer, which resides in certain procedure preliminary to the assembly of the cell, that is calculated to prevent action of the sal ammoniac on the manganiferous material while the cell is on the shelf.

20 By my invention I also make it possible commercially to utilize for battery manufacture, and more especially for use as a depolarizer, certain manganiferous materials which have hitherto not been used successfully in this art.

The invention also consists in other novel features hereinafter described and claimed.

The accompanying drawing shows a diagrammatic sectional view of a dry cell of 30 one type in connection with which my invention may be carried into effect.

I shall now describe one example indicating the manner in which the invention can be practiced.

35 In carrying out my process, I prefer to make use of a suitable tank of any appropriate size, shape and material, provided with a perforated or screenlike bottom. On the bottom of the tank is placed a suitable 40 piece of filtering material, such as cloth. The manganese compound which is to be employed, after having been ground or comminuted, and sifted, is charged into the tank, leaving a certain amount of space at 45 the top. A solution of a neutral salt usually an ammonium salt, for example, a solution of ammonium chlorid, of any appropriate density, say, one degree Baumé, is then poured into the top of the tank onto 50 the material and permitted to percolate through it. If it be assumed that the manganese material takes up, say, two-thirds of the tank capacity, the remaining one-third of the tank will be filled with the saline solution, which will pass completely into the 55 material under treatment in, say, twenty-four hours. Another similar quantity of the solution will then be poured into the tank and allowed to pass down into the material

60 in the same manner. After the lapse of forty-eight hours, for example, a third quantity of solution will be poured into the tank, and similar quantities of solution will be poured in at approximately equal 65 intervals, as needed. When the solution

commences to pass out of the tank at the bottom, the same is tested in any suitable manner which permits comparison with the solution being poured in at the top. I test the outgoing solution with a hydrometer 70 when the material being treated is a hydrate or a precipitate. When this grade of manganese material is treated, the increase in density will show strong contamination for the first passage of the liquid, but gradually 75 the impurities in the solution will thin out and a decrease of density is noted, until the solution coming out of the bottom of the tank has the same density as that poured in at the top. No further tests are then 80 needed. When the material being treated is pyrolusite, or natural manganese dioxid, for example, the solution passing out at the bottom, if its shows no difference in Baumé, 85 is tested chemically, which will indicate the character and amount of impurities, such as metallic oxids, which are being leached out. In any case, if the best results are to be obtained, the solution is passed through the material until that flowing out at the bottom 90 of the tank corresponds to that poured in at the top.

In this process, which will consume a variable length of time, depending on the kind of material treated, and the facilities 95 available, the impurities in the material which are soluble in the solution to be used in the assembled battery as an exciting agent, and especially those which render oxidation difficult, are separated out and removed in the outgoing solution. The manganese material, however, is not affected by the ammonium chlorid and remains in its original bulk.

The material remaining in the tank, 100 which is practically pure manganese oxids, is then taken out and dried and, if intended for use as a depolarizing material, is permitted to take up oxygen from the air. The amount of oxygen absorbed will, of course, depend to a certain extent on the amount of the lower oxids of manganese contained in the initial material. When the impurities have been removed, the material will 110 tend to absorb oxygen up to its full oxygen-absorbing capacity. It is preferable to expose the purified material to the air for several days at least, so that a maximum amount of oxygen will be taken up thereby 115 before it is used in the battery as a depolarizer.

In carrying out my process, I prefer to use a manganese precipitate as a starting material, or any cheap waste material containing manganese, but it will be understood from what has been said above that the process can be carried out successfully with more expensive grades of manganese. One of the particular advantages of my process, however, consists in the fact that 120 130

very cheap manganese containing materials, heretofore considered waste products, may be treated successfully and economically, whereby a superior depolarizer can be produced at a very low price compared to inferior depolarizers now used.

By my invention, very low grade material can be easily and economically converted into a high grade material which gives the very best results in the cell, increasing the E. M. F., and at the same time lengthening the life very considerably. The purified manganese material absorbs oxygen by a natural process, which is not only very inexpensive as compared to hydration and similar processes, but the product, containing substantially nothing but manganese and oxygen, and being in fact a very pure manganese dioxid, has much greater depolarizing efficiency than the substances commonly employed. The fact that the tests during the process of purification indicate that the ammonium chlorid used in the cell as an exciting agent will have no chemical effect upon the depolarizer, is also an important feature of advantage, as in this manner the possibility of any local action being set up from this source, is eliminated.

Obviously, the lowering of the cost of dry cells, by the use of low grade manganese-containing material, is a factor of no small importance. For example, I am able to use with entire success manganese compounds commonly occurring as waste products in the manufacture of permanganates, such as sodium permanganate, potassium permanganate and barium permanganate. In the oxidizing of manganates to produce such permanganates, there are precipitations of manganese compounds which can be purified to advantage by the above mentioned process for the production of a very satisfactory depolarizer. Other products which can be used are precipitations formed by agents used to remove the oxygen from permanganates. When oxygen is eliminated from a permanganate, for the purpose, say, of oxidizing, a precipitate is thrown down which has heretofore been considered practically worthless. If, however, the method previously described is used for the purification of a precipitate of this kind, it is a simple matter to recover all of the manganese. The impurities will be largely dissolved and removed by the ammonium salt in the manner previously described, and the resulting pure manganese material will take up oxygen, as above set forth, creating a manganese dioxid, which is very desirable for battery use. Cells made up with this material, showed on current tests, approximately 100% more life than standard cells of similar weight found on the market.

An example of a precipitate such as that above indicated would be a residue of potas-

sium permanganate which has been used in some industrial oxidizing process, which residue is thrown down as a basis manganese nitrate or sulphate, for example. This material is so finely divided as to be impalpable and usually has a dark blue color.

It is not necessary in all cases to expose such material to the air subsequent to its treatment by my purification process (with a neutral saline solution), for oxidation purposes, inasmuch as, with the impurities such as potash eliminated, it is exceptionally greedy in taking up oxygen from any available source, and the necessary oxygen for high oxidation is furnished it either from the substances used in mixing up the depolarizer cartridge or is taken up when the material is brought into contact with the electrolyte, on putting together the parts of the cell.

In my process above described, the density of the solution poured into the tank at various times should always be the same. That is, if I start out with a solution of one degree Baumé, subsequent quantities of the solution used are likewise one degree Baumé. It is not necessary to remove all of the sal ammoniac from the material before drying and oxidizing, if the material is to be used as a depolarizer. While it is possible to remove the sal ammoniac by washing with water, the material, as I employ it for battery purposes, carries a trace of sal ammoniac when placed in the cell.

In the drawing I have shown a sectional enlargement of a pocket dry cell in connection with the manufacture of which my invention has been practised with very good results. In this drawing, 1 denotes a zinc cup which serves as one electrode, and 2, a carbon rod serving as the other electrode. The depolarizing material, which may contain other ingredients in addition to the manganeseiferous material hereinbefore mentioned, is packed or rammed about the carbon electrode in such a manner as to form a cartridge 3 covered with cheese-cloth or like material 4. Within the space between the cartridge 3 and the side wall of the cup is a paste 5 carrying an exciting solution which, as above indicated, will usually be a solution of ammonium chlorid with or without the addition of zinc chlorid. The cell is closed at the top with sealing-wax 6 or the like, and between the top of the cartridge and the bottom of the closure 6 a paper washer 7 is interposed. It will be evident, however, from what has been said above, that it is not essential in all cases to have the same kind of solution with which the depolarizing material is treated for the removal of impurities, present later on in a paste within the cell, for while the invention has resulted in a marked increase in the efficiency of cells of this type, other types may be used.

Various changes and modifications may be made in the detailed procedure, and in other matters, without departing from the scope of the invention as defined in the 5 claims. For example, the process of treating the maganese material with an ammonium salt or salts may be considerably varied without departing from the broad principles of the invention; and if leaching of 10 the material with a neutral saline solution is practised, the method and means adopted for obtaining the leaching or lixiviating effect can be different from those herein particularly described.

15 I do not claim broadly herein a process for the purification of manganiferous material which comprises treatment of the material with a solution of a neutral salt, as claimed in my prior application hereinbefore identified. Neither do I claim herein the new depolarizer for electric dry cells or the method of making the same, or of making a cell containing a depolarizer around the carbon electrode, comprising recovered 25 manganese or, more particularly, a manganese derivative, as claimed in my application Serial No. 360,353; nor do I claim the dry cell per se as claimed in my application Serial No. 378,456.

30 What I claim is:

1. The method of making a primary cell, having a depolarizer, which comprises treating the depolarizer material, prior to the assembly of the cell, with a solution containing one or more of the salts used in the electrolyte, whereby deleterious substances soluble in the electrolyte are removed before the cell is assembled.

2. The method of making a primary cell 40 having a depolarizer and an electrolyte, which comprises treatment of the depolarizer with electrolyte material prior to the assembly of the cell for removing impurities that are soluble in the electrolyte.

45 3. The method of making a primary cell having a depolarizer and an electrolyte, which comprises as a preliminary step the leaching of the depolarizer with a solution containing electrolyte material prior to the 50 assembly of the cell.

4. The method of making a primary cell having a depolarizer and an electrolyte, such electrolyte consisting of or containing a neutral salt, which comprises the treatment of 55 the depolarizer material prior to the incorporation of the depolarizer in the cell, with a solution containing such neutral salt.

5. The method of making a primary cell 60 having a depolarizer and an electrolyte, such electrolyte consisting of or containing a neutral salt, which comprises the treatment of the depolarizer material prior to the incorporation of the depolarizer in the cell, with a solution containing such neutral salt, such

treatment being in the nature of lixiviation 65 and being continued until substantially all substances in the depolarizer soluble in the electrolyte are eliminated.

6. The method of making a primary cell 70 having a depolarizer and an electrolyte, which comprises leaching the depolarizing material with a solution of electrolyte material prior to the assembly of the cell, such solution of electrolyte material being of approximately the same concentration as the 75 electrolyte.

7. In the manufacture of primary cells, having a manganiferous depolarizer, the treatment of the manganiferous material 80 preliminary to its incorporation in the cell with a solution containing one or more of the ingredients of the electrolyte to be used in the cell, whereby the soluble impurities whose presence in the cell is deleterious to the life and strength thereof are removed 85 before the cell is put together.

8. The method of making a primary cell having a manganiferous depolarizer, which consists in leaching the manganiferous material prior to its incorporation in the cell 90 with a neutral solvent.

9. The method of manufacturing a primary cell having a manganiferous depolarizer and an electrolyte consisting of or containing a neutral salt, which consists in 95 leaching the manganiferous material prior to its incorporation in the cell with a solution of such neutral salt.

10. The method of making a primary cell having a manganiferous depolarizer and an 100 electrolyte consisting of or containing a neutral ammonium salt, which consists in so treating the manganiferous material, prior to the assembly of the cell, with such neutral salt that impurities in the depolarizer on 105 which such salt would act while the cell is on the shelf are eliminated before the parts of the cell are assembled.

11. The method of making a dry cell having a manganiferous depolarizer, a paste in 110 proximity thereto, and a saline exciting solution in the paste, which comprises the leaching of the manganiferous material with a quantity of such saline solution prior to the incorporation of such material in the 115 cell.

12. The method of making a dry cell having a depolarizer of manganiferous material, a paste in proximity thereto, and a solution of ammonium chlorid in the paste, 120 which comprises the leaching of the manganiferous material with a solution containing ammonium chlorid but devoid of acid for the removal of impurities soluble in an ammonium chlorid solution.

13. The method of making a dry cell having a depolarizer, a paste and a saline exciting agent in the paste, which comprises the 125

treatment of the depolarizing material with a neutral saline substance, in the absence of acid, for the purpose of removing deleterious substances.

5 14. In the manufacture of primary cells wherein ammonium chlorid is used as an exciting agent and a manganese oxid is employed as a depolarizer, leaching the man-

ganiferous material with a solution for the removal of impurities, and exposing the resulting depolarizing material to the air for oxidation prior to the assembly of the cell. 10

In witness whereof, I have hereunto set my hand on the 24th day of November, 1919.

HAROLD DE OLANETA.